

## United States Patent Office

3,556,710

Patented Jan. 19, 1971

1

3,556,710

**METHOD FOR BLEACHING TEXTILE FABRICS  
CONTAINING PORTIONS DYED WITH A  
SENSITIVE DYESTUFF**

Neil J. Stalter, North Minister, Wilmington, Del., assignor  
to E. I. du Pont de Nemours and Company, Wilmington, Del., a corporation of Delaware  
No Drawing. Filed Dec. 20, 1967, Ser. No. 691,970

Int. Cl. D06L 3/02

U.S. Cl. 8—111

8 Claims

**ABSTRACT OF THE DISCLOSURE**

Textile fabrics containing portions dyed with a sensitive dyestuff such as a vat dye, a naphthol dye or certain copper phthalocyanine dyes, are bleached by subjecting the fabric to the action of a bleaching solution containing a peroxyomonosulfate, which solution is buffered at a pH of 5 to 8.5, preferably a pH of 5.5 to 7. Bleaching temperatures up to about the boiling point of water are usable. Preferably, the fabric is saturated with such a solution and then bleached in the saturated state.

**BACKGROUND OF THE INVENTION**

The bleaching of textile fabrics containing portions dyed with a sensitive dyestuff has long been a problem. For example, when cellulosic fabrics containing portions dyed with naphthol dyes are bleached, the dyes have a marked tendency to bleed and "mark-off" onto the undyed portions of the fabric or onto other goods into which they may come into contact during bleaching. The tendency of such dyed portions to stain or mark-off is aggravated by severe bleaching conditions, particularly high temperatures, high alkalinites and extended bleaching times. Accordingly, mild bleaching conditions have been considered essential.

It has been proposed to bleach fabrics containing portion dyed with sensitive dyestuffs under mild conditions, e.g., at temperatures no higher than about 160° F. and pH values of from 6.5 to 10, as contrasted with the more severe bleaching conditions of temperatures of around 210° F. and pH conditions exceeding pH 10, such as are commonly employed when bleaching undyed cotton fabrics. Under such milder bleaching conditions, bleaching times of from about one-half to eight hours or more have generally been necessary. Patents indicating such prior practices are Kauffman U.S. Pat. 2,391,700 and Smollens U.S. Pat. 3,280,039. It has also been suggested (Prett et al. U.S. Pat. 3,227,655) that fabrics containing portions dyed with vat or naphthol dyes may be bleached with peracetic acid solutions at a pH of 4.5 to 6 and at temperatures of 60 to 90° C. However, the use of peracetic acid is distinctly disadvantageous because peracetic acid is a highly noxious and potentially hazardous chemical which generally must be manufactured at the mill site by persons inexperienced with its handling. Another distinct disadvantage in the use of peracetic acid is that it causes the discoloration of manganese-containing polyester fibers when the fabric being bleached is, for example, a blend of cotton and polyester fibers, such discoloration resulting from the reaction of the peracetic acid with residual amounts of manganese compounds present in polyester

2

fibers made by processes employing manganese compounds as polymerization catalysts.

Thus, there is a need in the textile industry for a simple process, preferably one that can be practiced continuously, for bleaching fabrics containing portions dyed with various sensitive dyes without requiring the subjection of the fabric to severe bleaching conditions and without incurring dye bleeding, staining, or mark-off onto the undyed portions of the fabric, and without incurring discoloration of polyester fibers containing residual manganese compounds. The present invention is directed to a process satisfying such a need.

**SUMMARY OF THE INVENTION**

A method for bleaching textile fabrics containing portions dyed with a sensitive dyestuff involving subjecting such a fabric to the action of a bleaching solution comprising an aqueous solution of a peroxyomonosulfate at a concentration to provide from 0.005% to 1% active oxygen, which solution contains a buffering agent effective to maintain the pH of the solution at a value within the range 5 to 8.5. Preferably, the fabric is saturated with such a solution and the saturated fabric is then heated, e.g., by steam, for a time of from 5 minutes to 20 hours to effect the bleaching.

**DETAILED DESCRIPTION AND  
PREFERRED EMBODIMENTS**

The bleaching solution employed in practicing the method of the invention is an aqueous solution containing a peroxyomonosulfate in an amount such as will provide in the solution a concentration of active oxygen of from 0.005 to 1%. Any of the water soluble peroxyomonosulfates such as the alkali metal peroxyomonosulfates, ammonium peroxyomonosulfate or the alkaline earth metal peroxyomonosulfates, can be employed. The most preferred peroxyomonosulfate is the potassium peroxyomonosulfate triple salt compound of the formula



A product comprising such triple salt compound and containing about 4.7% active oxygen by weight is available commercially. The peroxyomonosulfate component of the solution can also be formed in situ in the solution by the reaction of peroxyomonosulfuric acid, also called Caro's acid,  $\text{H}_2\text{SO}_5$ , and an alkali such as caustic soda, caustic potash, ammonium hydroxide or an alkaline salt such as sodium or potassium carbonate, or the like. Preferably, the concentration in the solution of active oxygen derived from the peroxyomonosulfate will range from 0.005 to 0.02% for immersion bleaching, and from 0.03 to 0.2% for saturation bleaching.

To be effective for the present purpose, the peroxyomonosulfate bleaching solution should be buffered to a pH within the range 5 to 8.5, preferably 5.5 to about 7. If the pH is lower than about pH 5, the solution may be sufficiently acidic to damage cellulosic fabrics. On the other hand, if the solution has a pH substantially higher than about 8.5, the solution becomes less stable. When the pH of the solution is buffered over the entire bleaching period to a value within the range stated, excellent bleaching of the undyed portions of the fabric, i.e., the white background portions, occurs with little or no bleeding of dyes from the dyed portions resulting and, conse-

quently, with little or no staining of the undyed portions or mark-off onto such undyed portions.

The commercially available peroxyomonosulfate triple salt product is quite acidic so that solutions thereof will generally require at least partial neutralization with an alkaline material in order to bring the pH of the solution within the range pH 5 to 8.5, most preferably 5.5 to 7. Such adjustment of the pH can be effected by the addition of any of the common alkalies such as sodium, ammonium or potassium hydroxide, or various alkaline salts, but it is also generally desirable that a salt having buffering properties such as to maintain the pH within such a range during the entire bleaching operation be also present. The alkali metal phosphates, particularly tetraalkali metal pyrophosphates such as tetrasodium pyrophosphate, are particularly effective for this purpose although other buffering agents such as sodium bicarbonate, the combination of borax and phosphoric acid or of tetrasodium pyrophosphate and sodium acetate may also be used.

Although bleaching with such solutions may be effected at ordinary temperatures, it generally will be preferred to employ somewhat elevated temperatures in order to decrease the bleaching time required. Thus, bleaching will generally be effected at a temperature of at least 100° F., e.g., temperatures from 100° F. up to as high as about 212° F. At such temperatures, bleaching times ranging from about 10 minutes to 5 hours may be employed, the higher temperatures generally requiring shorter times than lower temperatures. Bleaching may be effected by immersing the fabric in the bleaching solution maintained at the desired temperature, but preferably the fabric will be impregnated or saturated with an amount of the bleaching solution equal to from about 50% to 150%, preferably 80-120%, of the fabric weight, and the saturated fabric will then be heated at the desired temperature, e.g., by contacting it with live steam or a mixture of steam and air, depending upon the temperature desired. Most pref-

The invention is illustrated by the following examples in which all compositions expressed as percentages are by weight. Unless otherwise stated, the fabric samples employed in the examples were in tightly braided form and each sample was saturated with the designated bleaching solution and the saturated sample was then bleached in a chamber containing live steam or a mixture of live steam and air to get temperatures above 175° F., or placed in a covered beaker immersed in a water bath maintained at the desired bleach temperature to get temperatures below 175° F. Following bleaching, the samples were unbraided and rinsed well with hot water at least three times.

The following abbreviations are used in some of the examples to designate certain of the constituents of the bleaching solutions employed: DTPA designates a commercial diethylenetriaminepentaacetic acid sequestering agent; TSPP designates tetrasodium pyrophosphate decahydrate; and PMS designates the commercially available potassium peroxyomonosulfate product comprising the triple salt  $KHSO_4 \cdot K_2SO_4 \cdot 2KHSO_5$  having an active oxygen content of about 4.7%. Bleaching solutions containing peracetic acid were formulated using the commercially available 40% peracetic acid solution.

#### EXAMPLE 1

Samples of a cotton-polyester (ethylene glycol terephthalate) shirt fabric containing red stripes formed of yarns dyed with red disperse and naphthol red dyes, and black stripes formed of yarns dyed with black disperse and black vat dyes, woven into the fabric were bleached using the bleach solutions indicated in the tabulation below. Before bleaching, the fabric samples had been scoured by saturating them with an aqueous solution containing 0.83% TSPP and 0.5% soda ash, and then heating the saturated fabric at 150° F. for 60 minutes. The results obtained were as follows:

| Run | Bleach solution                                                                                                                            | Bleach conditions     | Bleeding or mark-off        |
|-----|--------------------------------------------------------------------------------------------------------------------------------------------|-----------------------|-----------------------------|
| A   | { 0.70% $H_2O_2$<br>1.25% sodium silicate<br>0.25% $NaHCO_3$<br>0.25% sulfonated castor oil<br>0.20% DTPA<br>0.02% Epsom salt<br>(pH 10.2) | 1 hour at 212° F.     | Considerable.               |
| B   | { 0.80% peracetic acid<br>0.40% TSPP<br>(pH 5.8 (NaOH))                                                                                    | 30 minutes at 210° F. | Visible but less than in A. |
| C   | { 1.0% PMS<br>4.0% TSPP<br>0.7% acetic acid<br>(pH 7.0 (NaOH))                                                                             | 15 minutes at 212° F. | None visible.               |

erably, a continuous length of the fabric to be bleached will be continuously saturated with the bleaching solution, following which the saturated fabric will be continuously heated by contact with steam or a mixture of steam and air and the heated fabric then stored, e.g., in a J-box or other equipment, from which it can be continuously withdrawn after a residence therein equal to the desired bleaching time.

The method of the invention is applicable to the bleaching of fabrics containing portions dyed with naphthol dyes, disperse dyes, vat dyes and copper phthalocyanine dyes. It is also applicable to fabrics containing one or more of the above type dyes and, thus, avoids the necessity of segregating differently dyed fabrics during bleaching. The process is suitable for bleaching the fabric in open width or rope form in the widely used continuous bleach J-box ranges with no significant modification of the equipment being required. Although continuous operation is most generally preferred, the method of the invention can be practiced in batch operations when desired.

Only a short bleaching time was required in Run C because essentially all of the active oxygen of the PMS salt was used up in that time. All of the samples were well-bleached, but the data show that only in the case of those bleached with the PMS bleaching solution did bleaching occur without causing the dye to bleed or mark-off onto the undyed portions of the fabric.

#### EXAMPLE 2

Samples of a light weight, all-cotton fabric containing a one-half inch check pattern dyed with a blue copper phthalocyanine dye were bleached with the bleaching solutions indicated in the following tabulation. White threads were pulled from each bleached sample and the extent of dye bleeding was assessed by observing the relative blue coloration of the white threads. The data tabulated below show that dye bleeding occurred to a significant extent when using the hydrogen peroxide or peracetic acid bleach solutions but did not occur to any significant extent when using the PMS type bleach solutions.

| Run | Bleach solutions                                                                         | Bleach conditions    | Relative coloration of white threads |
|-----|------------------------------------------------------------------------------------------|----------------------|--------------------------------------|
| A   | { 0.5% H <sub>2</sub> O <sub>2</sub><br>1.5% sodium silicate<br>0.06% Epsom salt         | 60 minutes at 210° F | Slight blue hue.                     |
| B   | { 1.0% PMS<br>1.5% NaHCO <sub>3</sub><br>(pH 6.7)                                        | 10 minutes at 210° F | None visible.                        |
| C   | { 1.0% PMS<br>1.5% Borax<br>2.5 cc. of 85% H <sub>3</sub> PO <sub>4</sub><br>(pH 6.2)    | do                   | Do.                                  |
| D   | { 1.2% PMS<br>2.0% TSPP<br>(pH 6.0 (H <sub>3</sub> PO <sub>4</sub> ))                    | 15 minutes at 210° F | Do.                                  |
| E   | { 0.23% peracetic acid<br>2.0% sodium acetate trihydrate<br>0.2% TSPP<br>(pH 5.8 (NaOH)) | 20 minutes at 212° F | Light blue hue.                      |
| F   | { 1.2% PMS<br>2.0% sodium acetate trihydrate<br>0.2% TSPP<br>(pH 5.8)                    | do                   | None visible.                        |

It is noteworthy that even when the PMS bleach solution contained a higher concentration of active oxygen than the otherwise similar peracetic acid bleach solution, (i.e., the PMS solution in Run F contained about 0.056% active oxygen whereas the peracetic acid solution in Run E contained about 0.048% active oxygen), the amount of dye bleeding was less with the PMS solution than with the peracetic acid solution. When the entire fabric samples were viewed, those bleached with the PMS solution had distinctly cleaner looking background portions than did those bleached with the other solutions.

When the general procedure of the above examples was followed in bleaching samples of a 50:50 cotton/polyester fabric having a red checked pattern (1/2" checks) containing disperse and naphthol red dyes, and the dye bleeding that occurred was assessed by observing the relatively pink coloration of white threads pulled from the bleached samples, it was noted that white threads from the samples bleached with alkaline peroxide solutions and peracetic acid solutions had visibly more pink coloration than did the white threads pulled from samples bleached with PMS solutions. Viewing the whole fabric samples, those bleached with PMS solutions had distinctly whiter looking background areas than did the samples that were bleached with alkaline peroxide or peracetic solutions.

#### EXAMPLE 3

Fabric samples similar to those in Example 2 were saturated with a solution containing 1% PMS, 0.5% TSPP and 2% sodium acetate trihydrate (pH 6.4) and bleached either at 120° F. for one hour in 2 stages or at 150° F. for 1 hour in a single stage. All of the samples were well bleached and there was no visible evidence of dye bleeding onto white background as compared to similar fabrics bleached with either alkaline hydrogen peroxide or peracetic acid bleaching solutions as indicated in the above tabulations.

#### EXAMPLE 4

This example illustrates bleaching in a continuous operation. Five samples of various colored fabrics, each about 6 ft. x 10 in., were butt-seamed together and the resulting assembly was butt-seamed into the center of a 100 yd. x 10 in. sample of unbleached, unscoured cotton fabric. The colored samples were: (a) a sample of the all-cotton fabric used in Example 2, (b) a sample of the cotton/polyester fabric used in Example 2, (c) an all-cotton light-weight fabric having a 1-inch red checked pattern dyed with naphthol red, (d) a medium weight all-cotton fabric having naphthol red stripes and yellow stripes against a broad white background, and (e) an all-cotton seersucker containing alternating 1/8" white and green

stripes dyed with a vat green dye. The resulting fabric train was continuously saturated to about 100% of its weight with a PMS bleaching solution of the composition set forth in Example 3, then bleached by passing it continuously through a J-box maintained at about 190° F. with a mixture of steam and air. The rate of travel of the fabric train through the J-box was such as to give a residence time therein for the fabric of about 30 minutes. The bleached fabric withdrawn from the J-box was washed by passing it through water at 180° F. following which the process was repeated. All of the colored fabric samples in the train were well-bleached and showed no evidence of bleeding or mark-off of the dye onto undyed portions of the fabric.

#### EXAMPLE 5

This example illustrates bleaching with a peroxymono-sulfate solution in accordance with the invention in a batch operation. Samples of a cotton seersucker fabric weighing about 11 grams and containing alternating white stripes and either stripes having yarns dyed with a vat blue dye or yarns dyed with a copper phthalocyanine dye, were bleached by immersing the samples for one hour in a solution maintained at 160 to 180° F. at a liquor:goods weight ratio of 10:1. The bleach solution contained 0.2% PMS, 0.5% TSPP and 0.3% acetic acid, and its pH had been adjusted to 6.2 with caustic soda. The bleached samples had well-bleached white backgrounds which showed no visible trace of dye bleeding or mark-off.

The fabric bleached in the above example contained many motes, some of which remained after the bleaching operation. This fabric was more difficult to bleach than were the fabrics used in the other examples and the fact that good bleaching of the white background was achieved demonstrated the bleaching effectiveness of the process of the invention. When samples of this same fabric were first given a mild scour (100% saturated with a solution containing 1% TSPP, 0.5% sodium carbonate and 0.1% of an anionic wetting agent, and heated at 180° F. for 30 minutes) and then bleached as indicated in Run F of Example 2, a well-bleached samples essentially free of motes resulted with no dye bleeding or mark-off being evident.

#### EXAMPLE 6

Samples of a cotton-polyester shirt material containing crisscrossing stripes of yarns dyed with either an orange dye, a gray dye or a naphthol red dye, were saturated with a bleach solution containing 1% PMS, 2% TSPP, and 0.5% acetic acid, its pH having been adjusted to 6.8 with caustic soda. The saturated samples were then heated at 180° F. for 15 minutes. This bleaching treatment caused

no dye bleeding or mark-off, nor any visible change in the color or hue of the dye.

Part of the above bleached samples were again bleached for 45 minutes at 210° F. using a bleaching solution containing 0.5% H<sub>2</sub>O<sub>2</sub>, 1.5% sodium silicate and 0.05% Epsom salt, the pH of the solution being 10.4. Although the white background areas of the re-bleached samples were well-bleached, the color of the dyed areas had been changed from the original bright red to a dull off-red. The remainder of the above once-bleached samples were bleached for 15 minutes at 210° F. with a bleach solution containing 1% PMS, 0.5% TSPP and 2% sodium acetate trihydrate, the pH of the solution being 6.4. The white background areas of the resulting twice-bleached samples were well-bleached and there was no visible change in the color of the dyed areas.

#### EXAMPLE 7

One-gram samples of an ethylene glycol terephthalate polyester yarn which contained residual amounts of a manganese compound polymerization catalyst were treated as indicated in the following tabulation with either a PMS bleach solution or a peracetic acid bleach solution.

| Run | Bleach solution                                                                                                      | Liquor: goods ratio | Bleach conditions   |
|-----|----------------------------------------------------------------------------------------------------------------------|---------------------|---------------------|
| A   | { 1.0% PMS<br>2.0% sodium acetate trihydrate<br>0.5% TSPP<br>pH 6.3<br>0.25% peracetic<br>0.5% TSPP<br>pH 6.3 (NaOH) | 20:1                | 150° F./1 hour.     |
| B   | Same as Run A                                                                                                        | 20:1                | Do.                 |
| C   | Same as Run B                                                                                                        | 1:1                 | 212° F./15 minutes. |
| D   | Same as Run B                                                                                                        | 1:1                 | Do.                 |

The samples treated with the PMS solution (Runs A and C) appeared essentially as white as the original untreated yarn, whereas the samples treated with the peracetic acid solution (Runs B and D) had an objectionable and distinct off-white cast. The results show that the PMS type bleach solution caused no significant discoloration of polyester fibers, containing residual manganese catalysts, whereas the peracetic acid bleach solution caused a distinct and objectionable discoloration. These results are significant since although polyester fibers per se ordinarily require little or no bleaching, such fibers are commonly blended in fabrics with cotton fibers which do require bleaching so that when blends of the two types of fibers are bleached, discoloration of the polyester fibers of the blend has the effect of decreasing the whiteness of the non-dyed portions of the fabric.

As indicated previously, the preferred peroxyomonosulfate bleach solutions for use in practicing the method of

the invention are slightly acidic. It might have been expected that such acidic solutions would have a degrading effect upon cellulosic fabrics. It has been found, however, that no significant degradation of such fabrics occurs when they are bleached with the PMS solutions indicated in the examples under the preferred pH conditions, i.e., pH 5.5 to 7. Thus, cotton fabrics bleached in single-stage operations under those conditions gave cuam values no higher than about 3. These are highly acceptable values since a cuam fluidity not exceeding about 7 is generally considered satisfactory.

I claim:

1. A method of bleaching a textile fabric having portions thereof dyed with a sensitive dyestuff, comprising subjecting said fabric to the action of an aqueous bleaching solution consisting essentially of a water-soluble peroxyomonosulfate at a concentration to provide from 0.005 to 1% active oxygen and a buffering agent effective to maintain the pH of the solution within the pH range of 5 to 8.5.
2. The method of claim 1 wherein the pH of the solution is 5.5 to 7.
3. The method of claim 1 wherein bleaching is effected by immersing the fabric in the bleaching solution at a temperature up to about 212° F., which solution contains 0.005 to 0.02% active oxygen.
4. The method of claim 1 wherein bleaching is effected by saturating the fabric with the bleaching solution containing 0.03 to 0.2% active oxygen, and maintaining the saturated fabric at a temperature from 100° F. to about 212° F. for from about 10 minutes to 5 hours.
5. The method of claim 1 wherein the fabric to be bleached has portions dyed with a naphthol dye.
6. The method of claim 1 wherein the fabric to be bleached has portions dyed with a vat dye.
7. The method of claim 1 wherein the fabric to be bleached has portions dyed with a copper phthalocyanine dye.
8. The method of claim 4 wherein the fabric is continuously saturated with the bleaching solution, the saturated fabric is continuously heated to a temperature of from 100° F. to about 212° F. and stored at said temperature for from about 10 minutes to about 5 hours.

#### References Cited

##### UNITED STATES PATENTS

- 3,048,546 8/1962 Lake et al. ----- 252—186X  
3,049,495 8/1962 Jenkins et al. ----- 252—186X

MAYER WEINBLATT, Primary Examiner

U.S. CL. X.R.

252—95, 99